

## UNITED STATES PATENT OFFICE.

JAMES C. MITCHELL, OF REYNOLDS, INDIANA

## EXPLOSIVE.

SPECIFICATION forming part of Letters Patent No. 783,844, dated February 28, 1905.

Application filed March 11, 1904. Serial No. 197,684.

*To all whom it may concern:*

Be it known that I, JAMES C. MITCHELL, a citizen of the United States, residing at Reynolds, in the county of White and State of Indiana, have invented certain new and useful Improvements in Explosives; and I do declare the following to be a full, clear, and exact description of the invention, such as will enable others skilled in the art to which it appertains to make and use the same, reference being had to the accompanying drawings.

My invention relates to explosives, and more particularly to gunpowders, and while more especially designed for both small and heavy arms, yet its application or use is not limited thereto where it can be otherwise effectively employed.

The object of the invention is to produce an explosive that will have high penetration power, that will not deteriorate or be detrimentally affected by changes in atmospheric conditions, that will be smokeless, that will not give forth or evolve harmful or noxious gases when exploded, that will not be exploded by concussion or jar in transportation or storage, that will cause the minimum of recoil in the gun when exploded, and that will possess other advantages.

In preparing the powder or explosive I mix together thirty parts of cane-sugar and ten parts of sugar of milk in an open vessel under heat until the mixture is brought to about boiling-point. It is then removed, and while still in a heated condition I add to it an extract of sandalwood—for instance, red sandal or saunders wood made by adding six parts of alcohol (preferably one hundred and eighty-eight proof) to four parts of the sandalwood distilled in an open vessel until an extract having more or less the consistency of a thick oil is formed. After the mixture has stood for a period of ten minutes, more or less, I add to the mass fifty parts of potash, (potassium chlorate.) The whole is then stirred until the ingredients become thoroughly incorporated or mixed. The mass is then dried in any suitable way sufficiently to permit trituration

and is then granulated by any suitable granulating or triturating means and is then ready for use.

By the use of the sandalwood treated in alcohol to produce the extract I find that the explosive is not detrimentally affected by atmospheric changes and that the particles maintain their granular form and will not again assume a plastic condition by the presence or action of moisture, which is ascribed to the sandalwood extract forming a protective coating insoluble in water. The powder can also be handled with perfect safety and without danger of explosion by concussion or jar during transportation. The explosive also possesses superior penetrating power and is smokeless and no poisonous or noxious gases are given off and the recoil is minimum. When the explosive is put up in the form of cartridges or shells and ignited or exploded in the usual way, it is found to leave no residue in the shell or cartridge or gun from which it is discharged and that whatever gas is evolved is consumed in the barrel of the gun, so that no noxious gases escape from the gun-barrel, as is common with many kinds of explosives heretofore made. From experiments made the advantages specified are ascribed to the presence of the sandalwood treated with alcohol to form an extract, and the advantages mentioned are based upon tests made with the explosive.

The theoretical composition of this explosive is given as follows: carbon, (C,) 22.18 per cent.; hydrogen, (H,) 3.44 per cent.; oxygen, (O,) 45.63 per cent.; potassium, (P,) 14.92 per cent.; chlorin, (Cl,) 13.53 per cent.; undetermined, .30 per cent. The undetermined .30 per cent. is attributed to the employment of the red sandalwood treated with alcohol in the composition.

The ignition-point of the explosive in an open bath is 188° centigrade—equivalent to 380.4° Fahrenheit.

From the foregoing it will be observed that the explosive has an oxygen-yielding substance—for instance, potassium chlorate—

the same being a chlorate of an alkali or alkaline chlorate; also, that it has carbonaceous substances, such as the milk-sugar and the cane-sugar, which constitute one group of carbohydrates, and also has a protective agent against the influences of moisture or water, the same being an extract of sandalwood insoluble in water, particularly the constituents of red sandalwood soluble in alcohol.

10 I have described with particularity the different ingredients and the proportions which I have found to give most satisfactory results based upon my experience in making the explosive; but I do not limit myself to the proportions nor to the particular ingredients where equivalent proportions and ingredients will produce substantially the same results; but in all cases the presence of the sandalwood extract is essential.

15 20 By the use of the phrase "extract of sandalwood" I do not mean to exclude the use of the cellulose of the wood, but use the phrase in the sense that it is the properties possessed by sandalwood that is made use of in the compound whether the cellulose of the wood be used or omitted.

While I have described a chlorate explosive powder, yet my invention lies in the discovery that the constituents of sandalwood soluble in alcohol serve as a preservative and protective agent against deleterious effect of moisture or water upon the oxygen-yielding and carbonaceous substances of an explosive powder in addition to security against accidental explosion and greater power of penetration believed to result from chemical changes due

to the presence of such extract in the composition.

Having described my invention and set forth its merits, what I claim is—

40 1. An explosive powder comprising oxygen-yielding and carbonaceous substances, and sandalwood extract insoluble in water, substantially as described.

45 2. An explosive powder comprising oxygen-yielding and carbonaceous substances, and constituents of red sandalwood soluble in alcohol, substantially as described.

50 3. An explosive powder comprising an alkaline chlorate and carbohydrates, and sandalwood extract insoluble in water, substantially as described.

55 4. An explosive powder comprising an alkaline chlorate, saccharine matter, and sandalwood extract insoluble in water, substantially as described.

60 5. An explosive powder comprising potassium chlorate, cane and milk sugars, and constituents of red sandalwood soluble in alcohol, substantially as described.

65 6. An explosive powder comprising cane-sugar, sugar of milk, potassium chlorate, and the constituents of red sandalwood soluble in alcohol, in substantially the proportions specified.

— In testimony whereof I affix my signature in presence of two witnesses.

JAMES C. MITCHELL.

Witnesses:

PARIS NORDYKE,  
WILLIAM GROSS.